

L. S. CHADWICK.

BURNER.

APPLICATION FILED NOV. 1, 1915.

1,247,792.

Patented Nov. 27, 1917.



FIG. 1.



FIG. 2.

INVENTOR,

Lee S. Chadwick  
Stull, Smith, Brock & West

Attys.

ATTY.

# UNITED STATES PATENT OFFICE.

LEE S. CHADWICK, OF EAST CLEVELAND, OHIO, ASSIGNOR TO THE CLEVELAND METAL PRODUCTS COMPANY, OF CLEVELAND, OHIO, A CORPORATION OF OHIO.

## BURNER.

1,247,792.

Specification of Letters Patent. Patented Nov. 27, 1917.

Application filed November 1, 1915. Serial No. 58,948

*To all whom it may concern:*

Be it known that I, LEE S. CHADWICK, a citizen of the United States, residing at East Cleveland, in the county of Cuyahoga and State of Ohio, have invented a certain new and useful Improvement in Burners, of which the following is a full, clear, and exact description, reference being had to the accompanying drawings.

10 This invention relates to that class of hydrocarbon burners involving what are known as commingling tubes that are arranged one within the other and between which gas rises from the burner proper and is burned, the tubes being perforated for the purpose of supplying oxygen required to promote proper combustion.

For obvious practical reasons, such as convenience and cheapness of manufacture, and because of its inherent tensile strength, steel has been found the most desirable material from which to make the commingling tubes.

It is acknowledged, however, by all familiar with this type of burner that the commingling tubes, especially the inner one, are very short lived. After a comparatively brief time, as a season to two of ordinary use, the tubes become distorted and brittle and actually collapse, while the remainder of the burner remains in practically perfect condition. It has been generally supposed that, by reason of the intensity of the heat under which they are 30 required to operate, the tubes have naturally become "burned out." This difficulty has been experienced for years, and so far as I am aware, no remedy has been suggested.

It is the object of my invention to obviate this difficulty in a simple and inexpensive manner and thus greatly increase the life of burners of this kind. In order that the real nature of the invention may be more readily understood and appreciated, I will 40 first explain the causes of the so-called "burning out" of the commingling tubes, and follow with a disclosure of how, by the exercise of my invention, the difficulty is overcome.

50 Considering the constituents of the hydrocarbons employed in burners of this character, and the physical characteristics

of the burner itself, it will be seen that a monoxid gas is produced between the commingling tubes, that is very rich in carbon.

In the operation of the burner, the tubes (especially the inner one, for it has not the cooling influence of surrounding low temperature air, as has the outer tube) are heated to a very high degree, approximately 1000° to 1200° F. We have, therefore, a situation analogous to that involved in the process of case-hardening steel, to wit, steel heated to a high temperature in the presence of carbon. At certain temperatures, iron in steel has a very strong affinity for carbon. When the commingling tubes acquire a given degree of heat, therefore, the iron in the tubes calls for carbon, the power of attraction increasing with the increase in temperature. The carbon in the gas that is between the tubes promptly responds to the call and in a comparatively short time the steel becomes so heavily charged with carbon that it has less strength than ordinary cast iron. In fact, the steel becomes so overcharged with carbon that it has very little more strength than the original iron ore, and may be pulverized under slight pressure. At this stage in the use of the burner the tubes bulge and crumble away.

It will be seen, therefore, that what we have is not a "burning out" of the tubes, but an over-carbonization of them, which renders them useless.

To prevent this carbonization of the steel, I coat or plate the commingling tubes with a substance impervious to carbon. In practice I have found copper a suitable material for this purpose for it has no affinity for carbon, and it may be economically and conveniently applied to the tubes by the well-known electro-plating process. Experiments have proven that commingling tubes so plated possess more than double the life of the plain steel tubes. Other materials than copper, which are practically unaffected by heat and are impervious to carbon, may be used in lieu of copper, and applied in any manner suitable to the circumstances. Therefore, my invention is not limited to the employment of any particular material for the coating of the tubes,

nor to the method of applying it, so long as the protective coating is effectual in excluding carbon.

5 A practical application of my invention is illustrated in the accompanying drawing, wherein—

Figure 1 represents a sectional side elevation of a hydrocarbon burner involving my invention; and

10 Fig. 2 is a highly magnified fragmentary section through one of the commingling tubes.

The drawing shows an ordinary burner of the class above discussed, the same comprising 15 inner and outer wick tubes 1 and 2, respectively, between which is confined the wick 3, the space between the wick tubes being supplied with liquid fuel through any suitable means. This form of combustion 20 device is selected merely for illustrative purposes, and the same may be displaced by any approved form, wick or wickless, that will properly coöperate with the commingling tubes. Supported above the combustion 25 device, in any suitable manner, as by having their lower ends resting upon the respective flanges 5 and 6 of the inner and outer wick tubes, are the inner commingling tube 10, and the outer commingling tube 11. 30 These tubes are shown as held together by rods 12 which cross each other substantially at right angles and at the center of the tubes and pass through the tubes, the protruding ends of the rods serving to sustain 35 the drum 13 which surrounds the commingling tubes.

It is apparent from the illustration that air, passing freely up through the drum about the outside of the outer commingling 40 tube, will serve to keep the temperature of this tube much below that of the inner one. In practice, this tube hardly reaches a temperature sufficiently high to cause it to absorb carbon and therefore the coating of the 45 outer tube may be dispensed with without serious consequences. However, I have shown both the inner and outer commingling tubes as coated with a substance impervious to car-

bon, the same being designated A in the drawings and illustrated in Fig. 1 by heavy, 50 solid lines, and in Fig. 2 by a stippled area.

It will be understood, of course, that the protective coating is applied to the commingling tubes after they have been perforated; so that the substance of the protective coating 55 may effectually protect every portion of the steel of the tube.

Having thus described my invention, what I claim is:

1. A commingling tube for burners of the 60 character set forth, said tube being coated with a substance preventing impregnation by carbon at high temperatures and the consequent destruction of the tube.

2. A commingling tube for burners of the 65 character set forth, said tube being coated with a substance impervious to impregnation by carbon monoxide at high temperatures, thereby preventing the destruction of the tube.

3. A commingling tube for burners of the 70 character set forth, said tube being formed of steel, and copper plated for the purpose of preventing the impregnation of said tube by carbon at high temperatures and the consequent destruction of said tube.

4. A commingling tube for burners of the 75 character set forth, said tube being formed of steel, and coated with a substance impervious to carbon at high temperatures for the 80 purpose of preventing the destruction of said tube.

5. A commingling tube for burners of the 85 character set forth, said tube being formed of a material comprising iron and coated with an electro-deposited substance preventing the impregnation of the tube by carbon at high temperatures and the consequent destruction of said tube.

In testimony whereof, I hereunto affix my 90 signature in the presence of two witnesses.

LEE S. CHADWICK.

Witnesses:

W. E. SHEPPARD,

BRENNAN B. WEST.